

Oct. 31, 1944.

L. H. WINKLER

2,361,672

STEEL WOOL

Filed April 3, 1940



*Steel Wool Containing C. under 0.35%  
and  
Metal of Group Consisting of Mn.,  
Mo. and Cr. 0.95 to 2.5%, the Balance  
being Substantially all Fe.*

Inventor

*Louis H. Winkler.*

By *R. S. A. Dougherty*  
Attorney

## UNITED STATES PATENT OFFICE

2,361,672

## STEEL WOOL

Louis H. Winkler, Bethlehem, Pa., assignor to  
Bethlehem Steel Company, a corporation of  
Pennsylvania

Application April 3, 1940, Serial No. 327,697

6 Claims. (Cl. 29—180)

My invention relates to an improved composition of steel for the manufacture of steel wool. This is made of relatively low carbon steel usually containing under 0.25 per cent carbon and up to about 0.85 per cent manganese. I have found that increasing the manganese content to a range from 0.90 to 1.5 per cent results in a decided improvement. With the increased manganese content the ease in machining required of this grade of steel to avoid excessive wear of the wool cutting knives is maintained and even increased. At the same time the fibres formed are longer, tougher, stronger and more uniform in all these respects. What is most important is that the resultant wool possesses the combination of soft and resilient characteristics most usually desired. The fibres are uniformly long and tough and not short and fragile. Because of the better quality of the wool produced, improved results are obtained in the operations of steel wool making such as winding, flattening, plaiting, compacting, forming skeins, braids, pads, etc. The individual steel fibres also have greater toughness and resilience contributing to the desired efficient scouring or cutting action in service.

It is not certain exactly why the increased manganese content aids in producing the soft and resilient type of steel wool which is generally desired, and which the trade finds difficulty in making, as against the harsh type of steel wool which is seldom desired and which can readily be made by certain adjustments in the wool cutting machines. Manganese is generally considered to have a hardening effect on steel rather than a softening effect; however, it may be suggested that perhaps in the somewhat tougher and harder higher manganese steel the fibres split off more readily ahead of the cutting tool. Furthermore, I have observed that the higher manganese steel has a more homogeneous microstructure with less banding and more uniform distribution of the carbides. The diameters of the fibres in the finer grades of steel wool approach microscopic dimensions and it may be conceived that a more homogeneous microstructure will produce a more uniform steel wool fibre. That is, as the fibres are cut off they are not seriously distorted and likewise not made fragile as might occur in steel of less favorable composition or structure. Hence the result is greater ease of machining and a softer wool with the improved physical characteristics described above. This conception of the desirable influence of improved

homogeneity was one of the factors leading to the study which resulted in this invention.

The occurrence of a more homogeneous microstructure is especially noticeable when the wire from which the steel wool is to be machined is patented wire of the higher manganese content. This patenting heat treatment has been found very beneficial for steel wool wire. Effective response of the steel to the patenting temperature gives a more homogeneous sorbitic microstructure with the carbides more uniformly distributed and with less ferrite banding. In wire with the higher manganese content of this invention I find better response to patenting. The beneficial effect of the higher manganese content on the microstructure, machinability, and hence on the quality of the steel wool, particularly softness and resiliency, is evident also in unpatented wire, but the best results are obtained when the higher manganese steel wire is patented.

I have found that molybdenum and chromium additions to the steel up to about 0.5 per cent, separately or together, have in general a similar improved effect to that of increased manganese content, and apparently for similar reasons. Molybdenum and chromium additions may be beneficially employed in conjunction with higher manganese. The manganese content may be held somewhat lower when additions of molybdenum or chromium or both are made, or as high a percentage of manganese may be used, as when molybdenum or chromium or both are not present.

The drawing shows a mass of steel wool, the showing being conventional so far as the wool structure is concerned. This drawing includes legends beneath the wool representation indicative of the field of compositions involved in the present invention.

The following are examples of compositions of Bessemer steel wire heats which have given decidedly improved results in the manufacture of steel wool:

| 45 | C        | Mn       | P        | S        |         |
|----|----------|----------|----------|----------|---------|
|    | Per cent | Per cent | Per cent | Per cent |         |
| 50 | .12      | 1.10     | .08      | .034     |         |
|    | .16      | 1.00     | .08      | .040     |         |
|    | .12      | .84      | .08      | .030     |         |
|    | .16      | 1.15     | .08      | .040     |         |
|    | .15      | .93      | .08      | .050     |         |
|    | .10      | 1.10     | .07      | .028     |         |
|    | .16      | 1.26     | .07      | .055     |         |
|    | .14      | 1.12     | .08      | .035     | .10% Cr |
|    | .10      | 1.25     | .07      | .030     | .10% Mo |

I have found it desirable to favor relatively low phosphorus content, preferably below 0.09 per cent phosphorus. I also favor relatively low sulphur content preferably below 0.05 per cent sulphur.

I have also found it advisable to employ considerable cold work by using greater percentages of reduction in drawing the wire from the rod than is conventional wire mill practice. This may be accomplished by drawing either on individual blocks or by continuous wire drawing equipment in which several dies are arranged in tandem. To obtain the best results careful technique in the wire mill must be employed; this contributes to the toughness of the wire and to the softness of final steel wool fibres.

Having thus described my invention, what I claim as new and desire to secure by Letters Patent is:

1. Steel wool containing under about 0.35 per cent carbon and from about 0.95 to about 1.5 per cent manganese and the remainder being substantially all iron.

2. Bessemer steel wire for the manufacture of steel wool containing under about 0.35 per cent carbon and from about 0.95 to about 1.5 per cent manganese and the remainder being substantially all iron.

3. Patented Bessemer steel wire for the manufacture of steel wool containing under about 0.35 per cent carbon and from about 0.95 to about 1.5 per cent manganese and the remainder being substantially all iron.

4. Steel wool containing carbon less than .35 per cent, and metal of the group consisting of manganese, molybdenum and chromium, in amount not less than .95 per cent and not greater than 2.5 per cent, the balance being substantially all iron.

5. Steel wool containing carbon less than .35 per cent, manganese in substantial amount up to 1.5 per cent, and molybdenum in substantial amount up to .5 per cent, the combined amounts of manganese and molybdenum being not less than .95 per cent nor more than 2.00 per cent, and the balance substantially all iron.

6. Steel wool containing carbon less than .35 per cent, manganese in substantial amount up to 1.5 per cent, and chromium in substantial amount up to .5 per cent, the combined amounts of manganese and chromium being not less than .95 per cent nor more than 2.00 per cent, and the balance substantially all iron.

LOUIS H. WINKLER.